

Feb. 18, 1936.

R. R. ROBINSON ET AL

2,031,070

METAL COATED ARTICLE AND PROCESS OF MANUFACTURE THEREOF

Filed May 17, 1933

*Fig. 1.*



*Fig. 3a.*



*Fig. 4.*



*Fig. 2.*



*Fig. 5.*



*Fig. 7.*



*Fig. 3.*



*Fig. 6.*



*Fig. 8.*



*Fig. 9.*

Robert R. Robinson  
Edward L. Rick Inventors

## UNITED STATES PATENT OFFICE

2,031,070

METAL COATED ARTICLE AND PROCESS OF  
MANUFACTURE THEREOFRobert R. Robinson and Edward L. Rick, Los  
Angeles, Calif.; said Rick assignor to William  
D. Howze, Los Angeles, Calif.

Application May 17, 1933, Serial No. 671,516

25 Claims. (Cl. 41—26)

Our invention relates to metal coated articles, and in particular to such articles as signs in which designs or characters are applied as a metallic overlay upon a base of wood fibre or similar cellulose material. The invention also relates to the process of producing such an article so as to enable it to withstand continued exposure without noticeable deterioration.

It is a particular object of this invention to provide a sign capable of use in the electrical industries for designating ownership of towers, danger and high voltage signs etc. Many of such signs are required by law, and must be placed in out of the way locations that make replacement difficult and expensive. Long life is therefore essential. Furthermore, as such signs are often made the target for hunters, as well as for small boys who delight in pelting them with rocks and shooting at them with rifles and airguns, they must sustain such misuse with minimum damage. Vitreous enamel signs often used for this purpose, shatter under such impacts, exposing the metal beneath, and destroying the readability of the sign. Such a sign as herein described of non-metallic body is of great value, as it will not cause radio interference, does not require grounding, and can be safely handled in high voltage fields. Small bulk and weight is another requisite, as repair wagons must carry 30 large quantities of these signs.

It is therefore an object of this invention to provide such a sign of thin section, of high insulation value and light weight, which will withstand the roughest sort of handling and misuse without material damage, which will be non-corrosive and permanent under all sorts of weather conditions and which will have a long life of readability.

A further object is to provide a process for the manufacture of such a sign and similar articles which will have the advantages above set forth, in particular whereby a wood fibre or similar surface may be prepared for the bonding thereto in a permanent manner of metals applied in molten state, and whereby the metal so applied will become an integral part of the body to which it is applied. A further object is the treatment of such a sign in a manner to eliminate the access of moisture to the bond surfaces, and to seal the body of the sign against subsequent moisture absorption. It is a further object to provide a unique method of preparing the surface of a cellulose body upon which metal is to be deposited whereby it will be free of moisture, oil, and other inherent and extraneous

substances or characteristics which could prevent proper bonding of the metal thereto.

Other advantages will be seen to obviously result from the provision of such a sign as described in the accompanying specification, and the process of manufacture thereof also described therein.

In the drawing, which shows but one embodiment of the invention and illustrates the various steps utilized in the process of producing such an embodiment:

Fig. 1 is a face view of a sign made in accordance with this invention.

Fig. 2 is a section taken on line 2—2 of Fig. 1.

Fig. 3 is an enlarged fragmentary view of the surface of the material used prior to treatment thereof.

Fig. 3a illustrates a method of preliminary surface treatment used on smooth surfaces of the body material.

Fig. 4 illustrates one method of heat treating the surface of the body material.

Fig. 5 illustrates the method used in applying the metallic lettering.

Figures 6, 7, 8, and 9 illustrate subsequent steps in the process of manufacture of the signs.

The body 11 of the sign is preferably composed of compounded wood fibre, one form of which is commonly known as "pressed wood" or "grainless wood". This material is manufactured from wood chips and shavings, exploded by steam into individual fibres, which are subsequently conditioned, graded, and recombined under heat and high pressure into highly compressed sheets. No binder is used, but the natural lignins and resins of the wood are brought out under the heat and pressure and serve as a binder. A paraffin oil is added for moisture-proofing. The sheets are pressed between smooth platens and wire screens, so that as received one side 11a is glazed and smooth, and the opposite side 11b rough, fibrous, and irregular in appearance, and covered with impressions 12 from the screen. This side is illustrated in Fig. 3.

Preparation of the surfaces for the reception of the metal lettering is therefore accomplished in two ways. When the smooth side is to be used, it is first subjected to a light sand blast as in Fig. 3a. Thereafter treatment of either side is the same.

The surface is next heat treated such as rapidly passing over the surface with an oxy-acetylene flame 13 as in Fig. 4. The intensely hot flame so obtained permits a rapid semi-carbonization of the surface, searing and thus sealing it with the

natural resins and lignins from the heated wood fibres; burning off the small fibrous fuzz on the rough surface as well as the sawdust and mill-dust, etc., which are present in varying amounts; 5 driving off the moisture and oils from the surface; all without allowing the heat time to penetrate into the material with sufficient intensity to injure the fibres inside. The surface is but partially carbonized, giving a permanent black-brown color, and is sufficiently changed in character from the somewhat soft, rough, fibrous original character of the surface to a dense, hard, resinous, oil and moisture-free base layer 11c, as to provide an ideal medium for the reception 10 of the subsequently applied metal.

Prior to such partial carbonization, each wood fibre on the surface is distinctly visible through a low power glass. Afterwards the separate fibers are not distinguishable even with a high power glass, the separate fibres seemingly having been 20 fused together into a compact, hard, surface. After a light brushing to remove the completely carbonized dust and fuzz, there is not sufficient free carbon in the surface to color a white cloth 25 rubbed over it.

Other treatments prior to heat treating are used for particular effects. For an intense brilliant black background, the surface is dampened with a sugar solution. Other substances can also 30 be successfully combined with the resinous surface during the heat treatment such as dyes resin-producing powders, and certain oils. In each case subsequent rapid, high temperature heating is used to properly change the character 35 of the surface for optimum bonding of the subsequently applied metal.

Other methods of carbonization than that illustrated may be used. Any extremely hot flame may be used, or a hot plate, heated by gas or 40 electricity, or a carbon arc. Chemical methods are also feasible, such as by sulfuric acid subsequently neutralized. The acetylene flame has been found practical and efficient in production work and is therefore illustrated, although it is 45 not desired to limit the heat treating process to any particular method.

After heat-treatment, the sign is lightly brushed or wiped to remove carbon dust, and then placed upon a jig board 14 having suitable 50 provision thereon for the locating of the sign body in conjunction with cooperating stencils 15 and 15a. A metal spray gun 16, with connections for oxygen, acetylene or hydrogen, and air, and supplied with metal in the form of wire, is utilized 55 to deposit metal through the stencils to form the metal lettering 17 upon the sign.

Stencil 15 is of paper or cardboard, and is held in close contact with the sign body 11, and retained against the forces of the gases from the 60 metal spray gun, by the metal stencil 15a. Suitable clamps, not shown, clamp the stencil 15a against the stencil 15 and the body 11 to the jig board 14. Centers of the various letters, such as the portion 18 of the "A" and 19 of the "o" 65 are covered by metal center pieces 21 supported on the bridging 20 of the metal stencil 15a. The openings in the metal stencil are slightly larger than the corresponding openings in the paper stencil 15, and thus allow for the collection 70 of metal particles on the metal stencil without interference with the sharp boundary line of the applied letters. The paper stencils are discarded after using two or three times. The center pieces 21 are cleaned by the operator when 75 metal collects upon them. The metal stencil is

partially protected by a resist such as soap or a thin oil or graphite.

The metal spray gun 16 utilizes the so-called Schoop process to deposit a thin coating of relatively impervious metal through the stencil openings. The gun is supplied with air at about 80 pounds pressure. The metal to be applied, in wire form, is fed into the heart of the oxy-acetylene flame. A blast of air is focused upon it at this point, atomizing the molten metal and carrying it at high velocity against the surface of the sign. The impact of the molten metal is sufficient to make it adhere tightly to the surface, keying itself into every crevice. A coating from two to five thousandths of an inch thick is used. Preferably, the lettering is aluminum, although zinc, tin, and other metals obtainable in wire form may be used.

Although the oxy-acetylene or oxy-hydrogen flame is used in this process, the material being 20 coated is not subject to high heat. The high velocity air blast keeps the material comparatively cool. The molten metal does not have time to cool and solidify between the melting point in the flame and its deposition on the material 25 and thus carries its heat directly to the point of impact. Careful examination of the product under the glass indicates that this heat is sufficient to slightly soften the surface previously "resinized" by the heat treatment, and that the 30 initial particles of molten metal actually imbed themselves into this surface. Other tests have shown that the metal cannot be mechanically removed without also taking away this resinized surface layer.

Cellulose compounds and wooden articles have heretofore been coated with metal by this Schoop process, after prior sand blasting. Results are very uncertain when attempting to apply coatings to wood, owing to the moisture, oils and resins in 40 the wood, and the gases formed in the wood when heated even by the air-cooled flame. By the herein described surface pre-heating process, coatings are applied to such surfaces without difficulty.

Further, such coatings as have been successful have been unbroken coatings, completely covering the wooden article to be coated. Intermittent coatings have not been successful, moisture being carried to the bond juncture of wood and metal 50 through the wood fibres and destroying what bond might there exist. Transparent protective oil, lacquer and varnish coatings are effective in excluding moisture only for a limited period. Shrinkage or expansion of the base material due 55 to moisture, freezing, and other atmospheric changes also will cause peeling of the metal coating.

The process herein described has produced metal coatings, which, unprotected by any oil, 60 varnish, lacquer or similar material, have withstood months of outdoor exposure without any visible deterioration. Such coatings were intermittent, such as the sign illustrated, in which there were areas of exposed heat treated wood 65 fibre surface adjacent the areas coated.

As a further protection and safeguard, after the metal lettering has been applied, the signs are soaked for a period of approximately thirty minutes in a sealing oil mixture 22, containing 70 linseed oil, soya bean oil, turpentine and other vegetable oils, known to the trade as "lionoil". This oil is of a thin consistency and readily penetrates the pores of the body material, and dries to a gummy, elastic consistency with fair rapidity. 75

Even when dry, it is still elastic and somewhat gummy and sticky. Suitable racks 22a are used to keep the signs separated during the soaking period, after which the racks are up-ended and the signs allowed to drain for about ten minutes as shown in Fig. 7. They are then wiped or squeezed such as by a slightly resilient wiper 23, (see Fig. 8) to remove the oil from the face of the metal letters and to distribute the excess oil along the edges of the letters and into the depressions in the face thereof where porous spots in the metal might occur. After such wiping the signs are hung on hook racks 24 for drying.

15 Since any moisture in the sign body 11 has been driven out by the pre-heating during carbonization of the surface, oil is absorbed into the pores from which the moisture was driven during the soaking process. The oil gums noticeably during the ten minute draining period, so that the subsequent superficial wiping removes but little oil except from the non-absorptive metal surface. A noticeable increase in transverse strength is obtained by the soaking in oil.

25 The sealing action of the oil is particularly advantageous along the edges of the letters such as at 25, Fig. 2. It is here if at all that defects in the metal application and bonding are apt to occur, such as are caused by paper particles from 30 the stencil 15, loosened by the air blast, adherence of the metal to the paper stencil, etc. As the metal is overlayed, there is a noticeable edge along each letter, and during the wiping, excess oil collects along this edge. The oil also will seep 35 through any porous spots in the metal coating, as at 26, and seal the pores beneath against the entrance of moisture.

Particular features of the material used are that, being compounded from short exploded 40 wood fibres, the fibres of the wood are not continuous, as in natural wood, and with the interstices between the fibres filled with oil, moisture is not transmitted through the body, even though it may enter the exposed edges. Consequently the 45 body does not check, crack, or weather as does natural wood. Likewise the screen depressions 12 provide a large key-hold for the sprayed metal as well as giving depressed areas of metal which tend to prevent serious injury from abrasion by 50 rubbing against each other during transportation, as well as from the sand-blasting action of wind blown sand in desert areas. The signs retain their readability, even though the high spots are abraded away.

55 Having thus disclosed our invention, we claim and desire to secure by Letters Patent:

1. A sign including a cellulose body and metallic indicia adhering to a surface thereof primarily through the intimacy of the contact therewith.

60 2. A sign including a cellulose body and metallic indicia adhering to a surface thereof primarily through the intimacy of the contact therewith, the cellulose material of said body being porous and a sealing compound impregnating the interstices of said body.

65 3. A sign including a body of compounded wood fibre having a portion of the volatizable matter removed from a surface of said body, and metallic indicia adhering to such surface primarily through the intimacy of the contact therewith.

70 4. The process of coating a cellulose body with metal which includes removing a portion of the 75 volatizable matter from the surface of said body

and subsequently directing molten metal particles thereagainst at high velocity.

5. The process of coating a cellulose body with metal which includes exposing a surface thereof to a high temperature and subsequently directing 5 molten metal particles thereagainst at high velocity.

6. The process of coating a cellulose body with metal which includes heating said body sufficiently to drive volatizable matter therefrom, directing 10 molten metal particles thereagainst at high velocity, and thereafter soaking said body in a sealing mixture.

7. The process of producing a sign which includes charring the surface of a wood fibre body, 15 directing molten metal particles thereagainst at high velocity while protecting certain surfaces thereof, soaking said body in a sealing mixture, and prior to the final drying thereof, redistributing the sealing mixture across the surface thereof.

8. A sign including a body of compressed carbonaceous material having a roughened surface, 20 said surface being partially carbonized, and metallic indicia adhering thereto primarily through intimacy of contact therewith.

25 9. A sign including a body of compressed carbonaceous material, having a roughened surface, said surface being partially carbonized, a portion of the volatizable matter normally in said body material having been expelled therefrom, metallic 30 indicia consisting of a relatively thin layer of metal upon said surface adhering thereto primarily through the intimacy of contact therewith, and a sealing oil impregnating said body and covering the surfaces of said sign.

35 10. A sign including a body of compressed wood fibre and indicia comprising a thin layer of aluminum adhering thereto primarily through the intimacy of contact therewith.

11. A sign as described in claim 10 impregnated 40 with a resinous oil.

12. The process of coating a carbonaceous body with metal which includes; roughening a surface thereof, partially carbonizing said surface, expelling moisture from said body, applying a thin 45 layer of metal thereto by melting said metal and atomizing the same into a high velocity spray directed against said surface, and soaking said body in a sealing oil.

13. The process of coating a carbonaceous material with metal which includes passing a high 50 temperature flame across the surface thereof, and subsequently directing a spray of molten metal against said surface.

14. The process of coating a material with 55 metal which includes applying a carbonaceous material to the surface thereof, carbonizing partly said last named material, and spraying molten metal thereagainst at high velocity.

15. The process of making a sign which includes coating the body thereof with a material 60 which bonds therewith and with subsequently applied metal under the influence of heat, subjecting the same to heat, and spraying molten metal thereagainst at high velocity to form metallic 65 indicia thereon.

16. A sign comprising a base of cellulose fibre, a portion of the volatile constituent thereof having been expelled from a surface thereof, and metallic indicia bonded to such surface primarily 70 through intimacy of contact therewith.

17. A sign as described in claim 16 and including a resinous oil impregnating such body and filling the interstices thereof from which volatile constituents have been expelled whereby the sub- 75

sequent access of moisture to the bonded surfaces of the body and indicia is prevented.

18. A sign including a body of cellulose fibre, said body containing on a surface thereof a series of depressions, metallic indicia overlying portions of said surface and having projections thereon corresponding with said depressions, said metallic indicia adhering to said body primarily through intimacy of contact therewith, the corresponding projections and depressions forming spaced anchoring points for each character of said indicia.

19. A sign comprising a base of cellulose fibre, and metallic indicia adhering to a surface of said body primarily through intimacy of contact therewith, said indicia being of such relative thinness as to appear after application substantially flush with said surface.

20. The process of coating a cellulose base article with metal which includes heating the surface to be coated at a high temperature for a relatively short time interval, whereby volatizable constituents are expelled from such surface without complete carbonization thereof, applying the

metal in a molten high velocity spray, and subsequently filling the interstices caused by such volatilization with a sealing oil by soaking the article therein.

21. A sign as described in claim 18 in which said surface is partially carbonized.

22. A sign as described in claim 18 in which said cellulose fibre has a portion of its volatile constituents removed and including a sealing material impregnating the interstices of said body from which such volatile material has been expelled.

23. A sign as described in claim 1 in which said surface is partially carbonized.

24. A sign comprising a body of fibrous insulating material and metallic indicia adhering to a surface thereof primarily through intimacy of contact therewith.

25. A sign as described in claim 24 and including a waterproof sealing material filling the spaces between the fibers of such insulating material.

ROBERT R. ROBINSON.  
EDWARD L. RICK.